

1,398,144.

E. E. NOVOTNY.

MANUFACTURE OF SOUND RECORDS.

APPLICATION FILED JULY 21, 1920. RENEWED MAY 3, 1921.

Patented Nov. 22, 1921.

*Fig. 1,*



*Fig. 2*



INVENTOR

Emil E. Novotny  
BY  
Mayers, Cavanaugh & Hyde  
His ATTORNEYS

# UNITED STATES PATENT OFFICE.

EMIL E. NOVOTNY, OF LOGAN, PHILADELPHIA, PENNSYLVANIA, ASSIGNOR TO JOHN STOGDELL STOKES, OF PHILADELPHIA, PENNSYLVANIA.

## MANUFACTURE OF SOUND-RECORDS.

1,398,144.

Specification of Letters Patent.

Patented Nov. 22, 1921.

Application filed July 21, 1920, Serial No. 397,926. Renewed May 3, 1921. Serial No. 466,534.

To all whom it may concern:

Be it known that I, EMIL E. NOVOTNY, a citizen of the United States, and resident of Logan, Philadelphia, in the county of Philadelphia and State of Pennsylvania, have invented certain new and useful Improvements in the Manufacture of Sound-Records, of which the following is a specification.

This invention relates to the manufacture 10 of sound records or disks such as are used in connection with phonographs and similar sound reproducing machines.

In this industry the desirability of making a record which, when played, will faithfully 15 and accurately reproduce the original tones with fullness, clearness and resonance, is well recognized. It is further appreciated that the degree of perfection in sound reproduction is dependent, to a great extent, 20 upon the physical characteristics of the body of the sound record itself. It has been found that if the body structure of a record is composed of what might be termed of a relatively soft, loose, or cellular mass, which is 25 lacking in hardness, compactness and density, there is a distinct tendency for the body of the record during the playing of the selection, to absorb the under-tones and over-tones, thereby failing in full and efficient 30 transmission through the stylus to the sound box. This results in faulty, dull, or subdued reproduction, particularly as to under-tones and over-tones which can be clearly heard 35 during the singing or playing of the original selection, but which practically disappear when the record is played. Numerous attempts have been made to produce a sound record of the requisite hardness and density to avoid the absorption of sound, as above 40 pointed out, but heretofore, so far as I am aware, efforts in this direction have not been successful for the reason that when a record of sufficient hardness and density has been made it has been found to be entirely too 45 brittle and frangible for practical purposes. In other words, the advantages obtained from the standpoint of hardness and density in the record have been more than offset by the fact that such a record will easily chip 50 or break, and will undergo attrition or rapid

wearing under the action of the stylus or needle, particularly when the latter is of steel. A steel stylus or needle will rapidly break off or destroy the thin, brittle minute walls of the sound grooves of the record thus 55 ruining the latter. Furthermore the exceeding brittleness of such a record renders it easily broken so that it has been heretofore practically impossible to make a record hard and dense enough to produce full and clear 60 under-tones and over-tones, and at the same time have it stand up under the wear and tear incident to handling and use.

With my invention however I am enabled to produce a hard, dense, compact sound 65 record which will clearly, faithfully and accurately reproduce original over-tones and under-tones, and which possessing strength and tenacity and lacking brittleness and frangibility is capable of withstanding 70 shocks and jars and the wear and tear occurring in service.

My invention consists in the construction, combination and arrangement of parts set forth in and falling within the scope of the 75 appended claims.

In the accompanying drawings:

Figure 1, is a cross sectional view of a blank such as is employed in making my 80 improved record.

Fig. 2, is a similar view of my complete record.

Before entering into a detailed description of my invention I will briefly state that in the manufacture of my phonograph record I select a porous base or body which may be in the nature of a fibrous substance. This I impregnate, short of the point of saturation, with a cementitious material which is capable of subsequent reaction to 85 assume a hard, set and preferably infusible form. For this cementitious substance I prefer to employ a synthetic resin preferably in the nature of a condensation product such as results from the reaction of a phenol and 90 an aldehyde. The impregnated fiber base or body is then so operated upon that the cementitious material is partially hardened and set, but not to such an extent as to render the same capable of further compres- 95 100

sion under molding pressure. In this condition I coat the impregnated base either on one or both faces with a cementitious material, such as the synthetic resin above mentioned, mixed however with a hardening substance such as barium sulfate. Under heat and pressure this coating will assume a very hard, dense and closely compacted form. This coating is intended to form an inner, 10 sound-repelling coating, for I apply or impose thereon an outer coating in which the grooves of the record are formed. This outer coating, which is also of a cementitious material such as the synthetic resin mentioned, is, however, softer and more tenuous than the barrier coating and of a more skin-like nature. Therefore, it is not as brittle as the barrier coating, nor as hard, and is not as susceptible to breakage but possesses 15 greater tensile strength and resistance to shocks and blows. The inner sound-repelling coating, by reason of its hardness and consequent brittleness, while it would not be well adapted for the outer coating of the 20 record because of its liability to breakage, yet serves admirably to prevent sound absorption by the fiber base, as it serves a barrier between the outer coating and such base. The result is that in the playing of 25 the record the over-tones and under-tones instead of being absorbed by the body of the record, are thrown outward by this inner or barrier coating and are transmitted through the stylus to the sound box, thus causing the 30 selection to be rendered in full, clear and resonant tones.

Referring now to the accompanying drawings in detail, and particularly to Fig. 1 which shows a blank or disk from which the 35 sound record may be made, the numeral 1 indicates the body or base which may be of any suitable material, but I prefer to have it composed of a porous substance, preferably of a fibrous nature such as felted paper 40 consisting chiefly of wood fiber, although I may utilize any open mesh material of suitable strength, even chip board or straw board. This base 1, I preferably impregnate, but not to the point of saturation, with 45 a minimum amount of cementitious material. This material is preferably in the nature of a synthetic resin such as a condensation product produced by the reaction of phenol and an aldehyde. For this purpose I may 50 use such well known commercial forms of phenolic condensation products as bakelite or condensite, or any suitable cementitious material capable of assuming a hard and set form. I use a minimum amount of the 55 cementitious material for impregnation purposes in order that the cellular structure of the fiber will be capable of compression, under molding pressure, without forcing any material quantity of the impregnated material 60 from its interstices. I prefer to subject the

impregnated fiber to a limited degree of heat, say from two hundred to three hundred degrees F., for from ten to sixty minutes, to partially harden or set the cementitious material after impregnation and to eliminate 75 all solvents thereby producing a prehardened body which is still capable of further compression as in the final molding of a record. The cementitious material, or condensation product with which the fiber is 75 impregnated is indicated at 2.

The impregnated base which is usually in the form of a disk may now be dipped in a bath composed of cementitious material, such as a synthetic resin or condensation product 80 above mentioned, mixed however with a suitable hardening material, such as barium sulfate, or metallic oxids, such as iron oxid or zinc oxid. If desired the mixture may also contain a suitable catalyst, such as nigrosin 85 or zinc chlorid, the catalyst being employed for the purpose of hastening the hardening and setting of the cementitious material. The mixture thus composed of the synthetic resin, the barium sulfate and the catalyst 90 may now be ground on a printer's ink grinding mill, a good mixture being one part of barium sulfate to two parts of phenolic gum carried in a solution of two parts of proper solvents such as alcohol, benzol, acetone or 95 the like. The dipping of the impregnated body 1 into the bath will result in the coating of such body, and after the dipping the article may be placed in a suitable oven, such as a vacuum oven, for the purpose of 100 driving off the solvent and of hardening and setting the coating which is indicated by the numeral 3. The coating 3, which is intended to form the sound-repelling coating to prevent absorption of the sounds by the body 105 or base 1, during the playing of the record, is not at this time hardened and set to its final, infusible form, but is still capable of taking an impression under molding pressure. At such stage the thus coated article 110 is provided with a second or exterior coating shown at 4, and which is applied by dipping the article in a bath composed of a synthetic resin, of varnish-like consistency which however contains a small percentage, of a 115 soft filler, such as lamp black, the proportion of lamp black employed being about twelve per cent. by weight of the phenolic gum used in the mixture of the outer coating. The material of the outer coating contains no barium sulfate, and therefore will not assume the same extremely hard, brittle condition of the inner coating 3. This outer coating is now dried in the oven to drive off the solvent and to partially harden and set 120 the coating to a non-flowing or skin-like consistency. The blank is now ready for the molding of the record, and this may be done in the usual manner by placing the blank 125 against the grooved face of a record matrix 130

and subjecting the same while so placed to heat and pressure in a suitable press to reproduce in the face or faces of the blank sound grooves 5 complementary to the elevations of the matrix, and at the same time to harden and set all of the cementitious material of the record to its final, hard, infusible form. In the complete record the result will be that the inner or sound-repelling layers 10 or coating 3 will be much harder and denser, but far more brittle than the outer coating or layers 4, the latter however being more tenuous, smooth and skin-like than the inner coating. This results in an ideal record, for 15 the inner hard coating 3 will prevent the absorption of sound by the body of the record during playing, while the outer coating being smooth and of great tensile strength will prevent the breaking or cracking of the 20 record under usage. At the same time the fibrous material of the base, reinforced and cemented by the impregnating material, will insure a tough and durable record which is 25 practically unbreakable and which may be dropped and stepped upon or otherwise subjected to violent usage without breaking.

If desired, in place of the synthetic resins or condensation products herein mentioned, I may use as the cementitious material, those 30 shellacs mixed with suitable fillers commonly employed in this art in the making of sound records, and therefore where I herein use the term cementitious material, I wish it to be understood as including such shellacs, or 35 other substances suitable for the purpose.

Furthermore instead of first impregnating the porous or fibrous body with the cementitious material, and then subsequently as a 40 separate operation applying the inner or sound-repelling coating thereto, I may impregnate the porous or fibrous body simultaneously with the application of this inner coating, this being done by dipping the fiber disks into a bath such as has been described 45 for the formation of the inner coating, continuing the dipping process for a sufficient length of time to permit of the material of the bath being absorbed by the cellular mass of the fiber until the proper degree of impregnation has been reached, at the same 50 time resulting in the deposit of a sufficient amount of the material of the bath upon the faces of the fiber body to form the coating 3.

It will, of course, be understood from the 55 above description that in the finished record, both the inner or barrier coating and the outer or grooved face coating are in a set, non-flowing condition, but the inner or barrier coating is harder and more brittle than 60 the outer coating, while the latter is more elastic and tenuous than the inner or barrier coating. Therefore, where I have in the claims used the expression "relatively soft", with reference to the outer coating, I do not 65 wish to be understood as conveying the im-

pression that this outer coating is in any manner plastic or pliable, but I wish to be understood as meaning that this outer coating is less brittle, but more tenuous and elastic than the inner coating, as before explained. 70

While I have herein shown and described a preferred embodiment of my invention, I wish it to be understood that I do not limit myself to all the precise details set forth 75 by way of illustration, as modification and variation may be made without departing from the spirit of the invention or exceeding the scope of the appended claims. 80

What I claim is:

1. A sound record comprising a supporting body having a grooved sound-reproducing face, and a sound-repelling barrier interposed between the grooved face and the supporting body. 85

2. A sound record comprising a body portion, a relatively hard, dense coating applied thereto and a relatively soft exterior coating imposed upon the hard, dense coating and having sound grooves formed therein. 90

3. A sound record comprising a body portion, a relatively hard dense cementitious coating applied to the body portion and a relatively soft, cementitious coating applied to the relatively hard coating and having 95 sound grooves formed therein.

4. A sound record comprising a body portion impregnated with cementitious material and having a plurality of coatings also of cementitious material, one of said coatings 100 being harder than the other, the softer coating having sound grooves formed therein.

5. A sound record comprising a fibrous body portion impregnated with a cementitious material, a relatively hard and brittle 105 coating applied to said body portion, and a skin-like coating relatively less brittle than the first mentioned coating, applied to the latter, said skin-like coating forming an exterior face of the record and having sound 110 grooves therein.

6. A sound record having a relatively hard cementitious coating containing barium sulfate, said sound record having a grooved face section. 115

7. A sound record comprising a body portion, a relatively hard cementitious coating containing barium sulfate applied to a face of the body portion, and a relatively soft coating formed of a hard and set synthetic 120 resin imposed upon the relatively hard coating and having sound grooves therein.

8. A sound record having a plurality of imposed coatings thereon, said coatings being composed of hard and set synthetic resinous 125 material, each coating differing in hardness from the other, the exterior coating having sound grooves formed therein.

9. The herein described method of making a sound record which comprises coating a 130

4  
body portion with a mixture of cementitious material and a hardening agent to produce a relatively hard coating, then applying a second coating of cementitious material to the first mentioned coating to produce a relatively soft skin-like coating and then subjecting the coated body to heat and pressure against a sound record matrix to harden and set the cementitious material and to produce sound grooves in the face of the article. 10  
Signed at New York city, in the county of New York and State of New York, this 14th day of July, A. D. 1920.  
EMIL E. NOVOTNY.